

## 1

3,356,548

SAFETY MINING EXPLOSIVE COMPOSITION OF NITRIC ACID ESTER OF A POLYHYDRIC ALCOHOL AND THE TERNARY MIXTURE OF AMMONIUM CHLORIDE, ALKALI METAL NITRATE, AND ALKALINE EARTH METAL CARBONATE  
 Adolf Berthmann and Paul Lingens, Leverkusen, Germany, assignors to Dynamit Nobel Aktiengesellschaft, Troisdorf, Germany, a corporation of Germany  
 No Drawing. Filed Sept. 1, 1966, Ser. No. 576,550  
 Claims priority, application Germany, Sept. 7, 1965,  
 D 48,143

8 Claims. (Cl. 149—66)

This invention relates to novel explosives. It more particularly refers to novel explosives which are gelatinous or plastic and are safer than known explosives.

Explosives are known which, in addition to one or more sensitizing components, also contain ammonium nitrate, ammonium chloride or calcium carbonate.

Upon the blasting of coal underground, gelatinous explosives must have a relatively high resistance to ignition by firedamp. Such explosives consist of a gelatinous phase (mixture of nitroglycerine and nitroglycol or diglycol nitrate thickened with nitrocellulose) and a solid phase of inorganic salts (ammonium nitrate and inert salts, for instance alkali chloride). These explosives, however, do not satisfy modern safety requirements with respect to the igniting thereof by firedamp. In order to obtain sufficient resistance to firedamp in accordance with the German Test for Explosives of Class I, a high content of inert salts (about 40% NaCl) must be added. Such explosives, therefore, have only a low specific energy as compared with ordinary gelatinous rock explosives. Furthermore, their behavior in the presence of heat is unfavorable.

It is an object of this invention to provide a novel explosive.

It is another object of this invention to provide an explosive particularly useful in coal mining.

It is a further object of this invention to provide an explosive which has increased deflagration safety.

It is still another object of this invention to provide an explosive which is safer with respect to firedamp ignition.

Other and additional objects of this invention will be

## 2

hydric alcohols such as glycol dinitrate, glycerin trinitrate, diglycol dinitrate, etc. However, mixtures of the said nitrates can also be used. It is preferred that the amount of gelatinous phase should be just sufficient to render the entire explosive composition gelatinous or plastic. Suitably, about 18 to 40 percent by weight of the explosive composition should be gelatinous phase, preferably about 25 to 35 weight percent.

According to this invention it is essential that the inorganic salt component consist of a combination of ammonium chloride, alkali metal nitrate and alkaline earth metal carbonate. The alkaline earth metals are exemplified by calcium, magnesium, barium or mixtures thereof. It is preferred to use calcium as the alkaline earth metal. The alkali metals are exemplified by sodium, potassium and lithium with preference being given to the first two named.

It has been found that the inorganic salt component of the explosive of this invention should contain the above named constituents in the following proportions:

Ammonium chloride: alkali nitrate 1-2:1 and preferably 1.2-1.7:1.

Ammonium chloride: alkali earth carbonate: 2-50:1 and preferably 5-25:1.

Alkali nitrate: alkali earth carbonate: 1-45:1 and preferably 3-15:1.

The replacement of the known salt mixtures of ammonium nitrate and sodium chloride by the ternary salt mixture of ammonium chloride, alkali nitrate and alkaline earth carbonate of this invention, leads surprisingly to an increase in the specific energy as well as to gelatinous safety mining explosives which have substantially more deflagration safety. The replacement of the known salt mixtures of ammonium nitrate, ammonium chloride and calcium carbonate by the ternary salt mixture of ammonium chloride, alkali nitrate and alkaline earth carbonate of this invention, leads surprisingly to an increase in the solids smoke components of the explosion products, and a lower explosion temperature and a product which meets the firedamp ignition standards according to German Test Provisions for Class I-Explosives.

The following Table I gives some thermodynamic properties of various explosives for purposes of comparison.

TABLE I

| Salt Mixture                     | Expl.-Heat<br>(kcal/kg.) | Expl.-Temp.<br>(°K.) | Smoke<br>Volume<br>(l./kg.) | Specific<br>Energy <sup>1</sup><br>(mt./kg.) | Solids<br>Smoke<br>Components<br>(Percent) |
|----------------------------------|--------------------------|----------------------|-----------------------------|----------------------------------------------|--------------------------------------------|
| 3NH <sub>4</sub> NO <sub>3</sub> |                          |                      |                             |                                              |                                            |
| 2NH <sub>4</sub> Cl              | I                        | 381.7                | 1,507                       | 751.5                                        | 45.4                                       |
| CaCO <sub>3</sub>                |                          |                      |                             |                                              | 24.8                                       |
| NH <sub>4</sub> NO <sub>3</sub>  | II                       | 142                  | 871                         | 394.7                                        | 13                                         |
| 2NaCl                            |                          |                      |                             |                                              | 59.7                                       |
| 5NH <sub>4</sub> Cl              |                          |                      |                             |                                              |                                            |
| 3NaNO <sub>3</sub>               | III                      | 268.9                | 1,304                       | 539.6                                        | 26.6                                       |
| CaCO <sub>3</sub>                |                          |                      |                             |                                              | 46.0                                       |

<sup>1</sup> The specific energy is the product of the gas constant R, the smoke volume in mols per kg. and the explosion temperature in °K.

come apparent from a consideration of this entire specification, including the claims appended hereto.

In accord with and fulfilling these objects, this invention includes a novel explosive composition which comprises a combination of a sensitizing component and an inorganic salt component. The sensitizing component is liquid or gelatinous and must be present in such an amount that the final explosive mixture is of a plastic or gelatinous nature.

Sensitizing components within the meaning of the present invention are the liquid nitric acid esters—or nitric acid esters thickened in known manner—of poly-

From Table I it can be noted that the specific energy of the salt combinations in accordance with the invention (III) is twice as high as the specific energy of (II). The solid smoke components of (III) are, furthermore, twice as great as those of (I). It is thus shown that, for instance, the salt combination of the invention in accordance with (III) has a relatively high energy and at the same time a relatively large amount of solid smoke components.

Testing for ignition of firedamp is accomplished with a series of charge columns 50, 40, 30, 20 and 10 cm. in

length. The tested explosive has the following composition in weight percents:

|                                                          |           |
|----------------------------------------------------------|-----------|
| Nitroglycerine/nitroglycol (60/40 weight ratio)          | 29%       |
| Gun cotton                                               | 1%        |
| Ca(NO <sub>3</sub> ) <sub>2</sub> (50% aqueous solution) | 3%        |
| Salt mixture                                             | Remainder |

It is another particular attribute of this invention that it avoids the use of ammonium nitrate. This is quite desirable because the exact grinding and the preparation of the ammonium nitrate are difficult to achieve due to the ease with which it takes up moisture and its low transformation point (32° C.).

It is within the spirit and scope of this invention to utilize a ternary salt mixture having a particle size such that at least 30% and at most 95% pass through a screen of 0.1 mm. openings.

The explosives in accordance with the invention can also contain known combustible substances (for instance, paraffin, sawdust) or else halogen-containing combustible substances (for instance, chloroparaffins, waxes having a base of chlorinated naphthalene). Of course, in such case it must be seen to it that there is present an amount of oxygen-producing inorganic salts of salt mixtures (for instance, NaNO<sub>3</sub> + NH<sub>4</sub>Cl in a molar ratio of 1:1) which is sufficient for the combustion.

Furthermore, known inert materials (for instance, sodium chloride, iron oxide, etc.) can also be added to the explosives of the invention.

The advantages of the safety mining explosives of the invention reside in the fact that the deflagration safety with simultaneous increase in the energy is improved as compared with the previously known safety mining explosives of Class I.

The practice of this invention is illustrated by the following examples which are in no way to be construed as limiting.

#### EXAMPLES 1a-b

Two explosives were prepared in known manner by mixing, the composition of the salts thereof being in accord with II and III of Table I above. The two explosives withstood a methane/air mixture when tested in accordance with the German Provisions for Safety Mining Explosives of Class I (see Mining Ordinance concerning the distribution of explosives in mining of Jan. 28, 1959; cf. also article by Ahrens, Nobel-Heft of May 1959).

#### (1a) Comparative example: Explosive in accordance with II of Table I above

Explosive consisting of:

|                              |                |      |
|------------------------------|----------------|------|
| Nitroglycerin                | percent by wt. | 17.4 |
| Nitroglycol                  | do             | 11.6 |
| Nitrocellulose               | do             | 1    |
| 50% calcium nitrate solution | do             | 3    |
| Ammonium nitrate             | do             | 26.5 |
| Sodium chloride              | do             | 40   |
| Sawdust                      | do             | 0.5  |

Explosive properties:

|                                        |                     |      |
|----------------------------------------|---------------------|------|
| Excess oxygen                          | percent             | +5.5 |
| Density                                | g./cm. <sup>3</sup> | 1.6  |
| Specific energy                        | mt./kg              | 45.7 |
| Detonation transfer lying free on sand | cm.                 | 7    |

Deflagration safety: If a cartridge of the explosive is heated in a furnace to 100° C. and if it is seen to by the use of a kieselguhr envelope that an accumulation of heat can take place in the cartridge, then at the end of 2 hours there is an increase in temperature in the explosive to about 700° C. This temperature is retained for a few minutes. Since as is known a methane/air mixture ignites at a temperature of 650° C. with an induction time of 10 seconds, firedamp igniting is to be expected if an

explosive of this type which is under the influence for some time of a hot smoke of a neighboring shot, is thereby caused to deflagrate.

#### 5 (1b) Explosive in accordance with the invention: Explosive in accordance with III of Table I above

Explosive consisting of:

|                              |                |      |
|------------------------------|----------------|------|
| Nitroglycerin                | percent by wt. | 17.4 |
| Nitroglycol                  | do             | 11.6 |
| Nitrocellulose               | do             | 1    |
| 50% calcium nitrate solution | do             | 3    |
| Sodium nitrate               | do             | 27.5 |
| Ammonium chloride            | do             | 28.8 |
| Calcium carbonate            | do             | 10.7 |

Explosive properties:

|                                        |                     |       |
|----------------------------------------|---------------------|-------|
| Excess oxygen                          | percent             | +0.85 |
| Density                                | g./cm. <sup>3</sup> | 1.58  |
| Specific energy                        | mt./kg              | 57.2  |
| Detonation transfer lying free on sand | cm.                 | 10    |

Deflagration safety: If a cartridge of this explosive is heated in a furnace to 100° C. and if it is seen to by the use of a kieselguhr envelope that an accumulation of heat can take place in the cartridge, there takes place then in the explosive by the end of 21 hours only an increase in temperature of about 245° C. At this temperature, a methane/air mixture will no longer be ignited.

30 A comparison of the above explosives shows that the composition in accordance with the invention has a 25% higher specific energy and favorable behavior with respect to heat. However, this behavior with respect to heat was definitely not to be expected in view of the large proportion of nitrates whose thermal decomposition can after all not be prevented by a substitution of the salts.

What is claimed is:

1. In a plastic and gelatinous explosive composition comprising about 18 to 40 weight percent referred to the explosive of a gelatinous component formed of at least one liquid, possibly thickened nitric acid ester of a polyhydric alcohol and an inorganic salt component; the improvement which comprises utilizing as the inorganic salt component a ternary mixture consisting of ammonium chloride, alkali metal nitrate and alkaline earth metal carbonate.

2. The improved explosive claimed in claim 1, wherein said ammonium chloride bears a mole ratio to said alkali metal nitrate of about 1 to 2:1; said ammonium chloride bears a mole ratio to said alkaline earth metal carbonate of about 2 to 50:1; and said alkali metal nitrate bears a mole ratio to said alkaline earth metal nitrate of about 1 to 45:1.

3. The improved explosive claimed in claim 1, wherein said ammonium chloride bears a mole ratio to said alkali metal nitrate of about 1.2 to 1.7:1; said ammonium chloride bears a mole ratio to said alkaline earth metal carbonate of about 5 to 25:1; and said alkali metal nitrate bears a mole ratio to said alkaline earth metal nitrate of about 3 to 15:1.

4. The improved explosive claimed in claim 1 containing, in addition to the named constituents, at least one oxygen liberating inorganic salt other than the aforementioned alkali metal nitrate and alkaline earth metal carbonate and at least one other explosive combustible substance selected from the group consisting of paraffins, sawdust, chlorinated paraffins and waxes having a base of chlorinated naphthalene.

5. The improved explosive claimed in claim 4 containing, in addition to the named constituents, at least one combustible chlorine-containing substance selected from the group consisting of chlorinated paraffins and waxes having a base of chlorinated naphthalene.

6. The improved explosive claimed in claim 1, wherein said inorganic salts have a particle size such that about

30 to 95 percent thereof will pass through a screen having 0.1 mm. openings.

7. The improved explosive claimed in claim 1, wherein said alkali metal is at least one selected from the group consisting of sodium, potassium and lithium.

8. The improved explosive claimed in claim 1, wherein said alkaline earth metal is at least one selected from the group consisting of calcium, magnesium, barium or mixtures thereof.

**References Cited****UNITED STATES PATENTS**

2,829,036 4/1958 Berthmann et al. 149—62

5 CARL D. QUARFORTH, *Primary Examiner.*

BENJAMIN R. PADGETT, *Examiner.*

S. J. LECHERT, JR., *Assistant Examiner.*